

Dec. 4, 1923.

1,476,448

C. O. JOHNSON ET AL

APPARATUS FOR AND METHOD OF HARDENING OR TEMPERING WIRE

Original Filed Feb. 24, 1920



Invessors  
C. O. JOHNSON  
C. H. JOHNSON  
by attorneys

Soule & Soule

Patented Dec. 4, 1923.

1,476,448

# UNITED STATES PATENT OFFICE.

CHARLES O. JOHNSON AND CHARLES D. JOHNSON, OF WORCESTER, MASSACHUSETTS.

## APPARATUS FOR AND METHOD OF HARDENING OR TEMPERING WIRE.

Application filed February 24, 1920, Serial No. 360,879. Renewed October 20, 1923.

*To all whom it may concern:*

Be it known that we, CHARLES O. JOHNSON and CHARLES D. JOHNSON, citizens of the United States, both residing at Worcester, in the county of Worcester and State of Massachusetts, have invented a new and useful Apparatus for and Method of Hardening or Tempering Wire, of which the following is a specification.

10 This invention relates to the bright hardening or bright tempering of wire, and particularly to that method according to which the wire is drawn first through a lead bath and then through an oil bath.

15 Although not particularly limited thereto this invention may be considered as an improvement over the invention of the said Charles O. Johnson set forth in his application for patent on apparatus for hardening 20 and tempering wire, Ser. No. 291,322, filed April 19, 1919, and we have shown it herein as being applied to that apparatus and the method disclosed in that application.

The principal object of this invention is 25 to provide for reducing the temperature of the lead bath through which the wire passes between the time at which it is subjected to the highest temperature and the time at which it is introduced into the oil so as to reduce any tendency of the lead to stick to 30 the wire and be drawn out of the lead bath with it.

The invention involves in its preferred form the provision of one or more baths or 35 compartments of molten lead, preferably located outside the ordinary furnace which is usually employed in hardening wire, the temperature of the said additional bath or baths being regulated so as to reduce it 40 finally substantially to the temperature at which lead melts, so that the wire will be drawn out of the lead into the oil bath at the lowest temperature possible.

Reference is to be had to the accompanying 45 drawings, in which—

Fig. 1 is a plan of a hardening and tempering apparatus constructed in accordance with this invention;

Fig. 2 is a longitudinal sectional view 50 of the same, the invention being shown, as stated above, as used in connection with the mechanism set forth in the above mentioned application, and

Fig. 3 is an enlarged longitudinal sectional view of the hardening apparatus.

As is well understood in this art, a plu-

rality of wires are led through the lead kettle or bath 10 of a hardening furnace 9 where the wire is subjected to the highest degree of heat necessary to accomplish the well known result.

According to this invention the lead kettle or bath 10 occupies the usual position in the furnace 9 and is of a length substantially the same as the length of the furnace. We have shown this as being supplemented by two additional lead baths or compartments 12 and 13. These are heated in any desired way, as for example, by gas or oil burners 14 and 15 which can be regulated to any desired degree. It is important that the bath or kettle 13 should be heated only just a little above the melting temperature of lead so as just to keep the lead in a molten condition and not superheat it above that state, while the bath 12 is kept at a temperature intermediate between that and the temperature of the bath 10 in the furnace. This is controlled by the regulation of the burners 14 and 15.

Although we have described these three baths as separate we prefer to form them from a single casting in the form of a pan or kettle 16 which is divided by partitions, as for example, 17, 18 and 19 to provide the several compartments. We have also shown the kettle or compartment 12 as comparatively narrow, the kettle or compartment 13 being about 50% wider than the narrow kettle 12. The latter is shown as approximately a quarter of the length of the main kettle 10. These partitions are provided with grooves 20 in their upper surfaces for allowing the wire to pass from one to the other in a straight line always under the surface of the metal so that they have no access to the air.

At the point where the steel wire passes from the bath 13 to the cold oil bath 21 the wire is protected also from contact with the open air. The bath 13 is kept substantially at the melting point of lead and for that reason as the wire passes from the lead to the oil the carbonization of the oil by the heated wire, so common in this art, and also the lead pulling, does not take place and the smoke and fumes ordinarily encountered are substantially eliminated. The last wall 19 is provided with slots 22 through its upper surface which extend down to a level below the normal level of the molten lead in that compartment. The grooves or slots

22 are of a size adapted to the size of the wire and they allow the molten lead to stand in them as the wire passes through. The molten lead does not wet or stick to the 6 walls of the grooves and the low temperature to which it is brought assists in preventing this. It does not run out through the grooves because of the natural repulsion between the surfaces of the iron walls of the kettle 10 and the molten lead and because the grooves are near the surface of the lead bath. Furthermore the oil at a lower temperature meets the lead in the grooves and repels it. As will be seen it also flows over a grooved 15 dam 23 in a direction to force back any lead in a free condition located in these grooves. Although we mention lead and oil the invention is applicable to any other suitable heating and cooling liquids.

20 A space 25 is provided between this dam and the wall 19 for receiving the oil as it flows over the dam and waste pipes 26 are provided for introducing the oil therefrom into an oil tank 27 below, said pipes extend 25 below the level of the oil in said tank so as to exclude air from entering said pipes. The oil in the tank 21 is kept at such a level by any desired feeding apparatus and an overflow 29 as to cause it to constantly flow over the dam. This dam is provided with slots 28 in its upper edge or apex for receiving the wires directly from the slots 22 in a straight course. This is to cause the wire to pass through in a straight line without exposure to the air, being covered by the lead until the instant at which it enters the oil.

The dam is adjustable and held in position by means of screws 30.

40 It will be noticed also that on account of the flow of the oil in a direction the reverse of that of the motion of the wires there is a tendency to prevent its temperature from being raised excessively by the wire.

45 The above description is of the hardening apparatus, but the tempering apparatus 39 is constructed in substantially the same way except that the tempering lead bath 40 is not necessarily located in a covered furnace 50 because the temperature of the lead bath is lower, but additional lead baths 41 and 42 are employed and heated to a still lower temperature by gas jets 43 below or in any other desired way.

55 In this way not only is the wire prevented from being exposed to the air during the hardening process and also during the tempering process, but it is introduced into the oil at a reduced temperature, thus preventing the lead from sticking to the wire and being carried over into the oil, producing combustion of the oil by its contact with the heated wire. The uniformity, strength and temper of the wire are all improved.

60 Although we have illustrated and de-

scribed only a single form of the invention and shown it as applied to the invention illustrated in the above identified application, we are aware of the fact that modifications can be made, and that it can be applied 70 to other hardening and tempering devices by any person skilled in the art without departing from the scope of the invention as expressed in the claims. Therefore we do not wish to be limited to all the details 75 of construction or to the specific type of hardening and tempering apparatus herein shown and described, but what we do claims is:—

1. In an apparatus for treating wire, the 80 combination with a lead heating bath and an oil cooling bath, of an intermediate lead bath between them kept at a temperature below the temperature of the first named lead bath and means for guiding the wire 85 through said baths in a substantially straight line below the surface of the lead in each lead bath.

2. In an apparatus for treating wire, the 90 combination with a heating bath and a cooling bath, of an intermediate bath between them kept at a temperature below the temperature of the first named bath, and a partition between the heating and intermediate baths having a passage for the wire located 95 below the level of the liquids therein.

3. In an apparatus for hardening or tempering wire, the combination with a molten lead heating bath, a bath of molten lead maintained substantially at the melting point 100 of lead, a lead bath between them kept at an intermediate temperature and a cooling bath.

4. In an apparatus for hardening or tempering wire, the combination with a molten lead heating bath, a bath maintained substantially at the melting point of lead, a bath between them kept at an intermediate temperature, a cooling bath of oil, and means for guiding the wire through said 110 baths and for keeping it out of contact with air as it passes from one to the other.

5. In an apparatus for hardening and tempering wire, the combination of a comparatively long molten lead heating bath, a bath of molten lead maintained substantially at the melting point of lead, and substantially shorter than the heating bath, and an intermediate bath shorter than either.

6. The method of bright hardening or bright tempering of wire, which consists in passing the wire from a lead bath maintained at the usual hardening or tempering temperature into a second lead bath maintained at a lower temperature, then into a third lead bath barely maintained at the melting temperature of lead, and then directly into an oil bath and keeping the wire immersed in each bath until it enters the next one to prevent contact with air.

7. The method of hardening or tempering steel wire which consists in immersing it in a bath of molten metal, then reducing its temperature while still submerged in molten metal and without changing its direction of motion and finally passing it through a cooling bath.
8. The method of bright hardening and bright tempering of wire which consists in passing the wire through a plurality of connected baths of molten metal of varying temperature directly into a connected oil bath and keeping the wire immersed in each
- 15
9. In an apparatus for hardening and tempering of wire, or either, the combination of a plurality of molten metal baths of varying degrees of heat, with an oil bath directly connected therewith and means for 20 keeping the wire submerged in each bath until it enters the next.

In testimony whereof we have hereunto affixed our signatures.

CHARLES O. JOHNSON.

CHARLES D. JOHNSON.